

## UNITED STATES PATENT OFFICE.

NAPOLEON PETINOT, OF NEW YORK, N. Y., ASSIGNOR TO UNITED STATES FERRO-ALLOY CORPORATION, OF NEW YORK, N. Y., A CORPORATION OF NEW YORK.

## PROCESS OF MANUFACTURING ALLOY STEELS IN ELECTRIC FURNACES.

No Drawing.

Application filed November 16, 1922. Serial No. 601,407.

*To all whom it may concern:*

Be it known that I, NAPOLEON PETINOT, a citizen of the United States of America, and a resident of the city, county, and State 5 of New York, have invented a certain new and useful Process of Manufacturing Alloy Steels in Electric Furnaces, of which the following is a full, clear, and exact description.

10 This invention relates in general to the production of alloy steels in electric furnaces, and more particularly to low carbon alloy steels such as chromium, tungsten, manganese, vanadium, and other alloy steels 15 having a low carbon content. In carrying out my process, I employ an electric furnace.

It has heretofore been a practice of the art in making low carbon alloy steels in electric furnaces to first make a plain carbon 20 steel low enough in sulphur and phosphorus to comply with the specifications for such elements, and then to add enough of the ferro-alloy to bring up the content of the steel bath, as regards the alloying element, 25 to the desired percentage. Since all ferro-alloys contain more or less carbon, this carbon will be taken up by the molten steel. For this reason, therefore, it has been necessary to make allowance for the carbon, and 30 when a low carbon alloy steel was required, it was exceedingly difficult and in some cases impossible to produce the alloy steel with the desired low carbon content. In any such case, a very low carbon ferro-alloy must 35 be used, and this practice is expensive since such ferro-alloys are costly.

By using my invention, alloy steels of low carbon content (for example from 0.05% of carbon and upwards) can be made without 40 using low carbon ferro-alloys for the purpose of introducing the alloying substance.

Some of the objects of my invention have been to simplify the present methods of the art in the production of low carbon ferro-45 alloys; to reduce the cost of manufacture of such alloys; to do away with using low carbon ferro-alloys for introducing the alloying substance; and to do away with the use of burnt lime for the formation of the carbide 50 acting as a reducer.

In carrying out my invention, I make a bath of iron with a low carbon content in an electric furnace of the arc type and preferably in a basic lined furnace of such type. 55 This is easily accomplished by melting cold

scrap in the furnace, or transferring hot metal into the furnace from a basic open-hearth furnace. When the bath of steel is formed in the electric furnace and the first slag (a term well understood by those skilled in the manufacture of steel by means of an electric furnace) removed, I then add the ore of the metal which it is desired to combine with the iron. For example, if I desire to make a chrome steel out of various 60 chromium contents, then after the bath of steel has been formed in the electric furnace as above described, and the first slag removed, I then add chrome ore in a ground form. The following analysis is a typical 65 one of such chrome ore:

|                       | Per cent. |
|-----------------------|-----------|
| Sesquioxide of chrome | 48 to 56  |
| Silica                | 1 to 2    |
| Alumina               | 7 to 15   |
| Magnesia              | 13 to 16  |
| Iron oxide            | 14        |

After such ground chrome ore has been added, the current is again applied to the furnace, sufficient in quantity to melt the 80 contents, and thereby a chrome slag is formed. The slag is then carburized by an addition of some carbonaceous matter such as coke dust, petroleum coke, anthracite coal, carbon electrodes or the like. There is then 85 immediately formed carbides of lime aluminum, magnesium, etc., and the oxide of chromium and iron will be reduced to their metallic form, and will be absorbed by the bath of steel.

If a tungsten steel were desired, there 90 would be used in place of the chrome ore the calcium salt of tungsten, known as schelite. This schelite having been ground would be added to the bath of steel, and then after 95 the first slag was removed, the slag is carburized as above set forth. The result in this case would be that the tungsten formed would be absorbed by the steel, leaving a 100 slag of carbides in which the element, calcium, would predominate.

From the foregoing description, it will 105 be plainly seen and understood that my process, as herein described, is readily applicable to the production of other alloys such as vanadium, manganese, and the like, and that the production of such other steels will be attended by as advantageous results as those which follow from the production of chrome and tungsten steels, as herein 110

more specifically described. In other words, it will be clear to anyone skilled in metallurgy how my invention can be applied in the production of any alloy steels of low 5 carbon content.

Having thus described my invention what I claim is:

1. A process of making alloy steels in electric furnaces comprising the formation 10 of a bath of iron having a low carbon content in an electric furnace, then forming a slag with the impure ore of the metal to be reduced, and then carburizing the slag.
2. A process of making alloy steels in electric furnaces comprising the formation of a 15 bath of steel, then removing the first slag, then the formation of a slag with the impure ore of the metal to be reduced, and then carburizing the metallic slag thus produced.
3. A process of making alloy steels in electric furnaces comprising the formation of a 20 bath of iron, having a low carbon content, in a basic lined furnace of the arc type, then forming a slag with the impure ore of the metal to be reduced, and then carburizing 25 such metallic slag.
4. A process of making alloy steels in elec-

tric furnaces comprising the formation of a bath of iron having a low carbon content, then removing the first slag, then forming 30 a slag with the impure ore of the metal to be reduced, and then adding a layer of carbonaceous material in powder form, whereby the metallic slag is carburized.

5. A process of making alloy steels in electric furnaces comprising the formation of a 35 bath of iron having a low carbon content in an electric furnace, then removing the first slag produced, then adding chrome ore in a ground form, and then forming a 40 chrome slag.

6. A process of making alloy steels in electric furnaces comprising the formation of a 45 bath of iron having a low carbon content in an electric furnace, then removing the first slag produced, then adding chrome ore in a ground form, then forming a chrome slag, and then carburizing the chrome slag by adding a layer of carbonaceous material 50 thereto.

In testimony whereof, I have hereunto signed my name.

NAPOLEON PETINOT.